

# UNITED STATES PATENT OFFICE.

JAMES R. ROSE, OF EDGEWORTH, PENNSYLVANIA, AND JOHN HARRIS, OF LAKEWOOD, OHIO, ASSIGNEES TO CARBO-OXYGEN COMPANY, OF PITTSBURGH, PENNSYLVANIA, A CORPORATION OF DELAWARE.

## GASEOUS FUEL.

1,404,224.

Specification of Letters Patent. Patented Jan. 24, 1922.

No Drawing.

Application filed December 26, 1919. Serial No. 347,451.

To all whom it may concern:

Be it known that we, (1) JAMES R. ROSE, (2) JOHN HARRIS, citizens of the United States, residing at (1) Edgeworth, (2) Lakewood, in the county of (1) Allegheny, (2) Cuyahoga, and State of (1) Pennsylvania, (2) Ohio, have invented a certain new and useful Improvement in Gaseous Fuel, of which the following is a full, clear, and exact description.

This invention relates to gaseous fuel, and more particularly to a fuel which is especially adapted for the purpose of cutting metals with great rapidity, where extreme cleanliness of cutting is not essential. A use for which our gas is particularly well suited is for cutting scrap iron.

We obtain a gas having the above desirable characteristics by mixing with hydrogen, as a combustible base, butane and carbon monoxide in the proportions of from 2½% to 12½% by volume each of such butane and carbon monoxide to the hydrogen constituent. The carbon monoxide serves to increase slightly the temperature produced by the combustion of hydrogen alone. Furthermore, the gaseous mixture produces with in the burning hydrogen a visible cone which enables the operator to adjust the proportions of the gases and the combustion-supporting oxygen as may be necessary and to apply the flame in the most advantageous manner to the work. Both the volume of the flame and the heat units produced by the combustion of the mixture are greater than are produced by the combustion of hydrogen alone but are lower than usually required for operating on heavy masses of metal and for cutting cast iron and steel and corroded, dirty and slaggy iron and steel. However, our gaseous mixture is capable of

cutting with much greater rapidity than can be accomplished by gases having such higher carbon content.

According to Richards on Metallurgical Calculations, published in 1908, the flame temperature produced by the combustion of the aforesaid gases will be above 3200° C., and the variations in the percentages of the said gases will cause approximately the following variations in the net B. T. U. per cubic foot of mixture and in the cubic feet of oxygen required for the combustion of a cubic foot of such mixture:

No. 1 mixture, 95% H. with 2½% each of butane and carbon monoxide; net B. T. U.'s 368; cu. ft. of oxygen .650.

No. 2 mixture, 75% H. with 12½% each of butane and carbon monoxide; net B. T. U.'s 659; cu. ft. of oxygen 1.250.

Having thus-described our invention what we claim is:—

1. A gas for cutting, welding and heating purposes consisting of a mixture of carbon monoxide and butane with hydrogen in the proportions of from 2½% to 12½% by volume each of carbon monoxide and butane to hydrogen.

2. A gas for cutting, welding and heating purposes consisting of a mixture of butane and carbon monoxide with hydrogen in proportions not substantially less than 5% by volume of such combined gases to the hydrogen and not materially more than 25% of such combined gases to the hydrogen, the butane and carbon monoxide being present in the proportions of at least 2½% each in such mixture.

In testimony whereof, we hereunto affix our signatures.

JAMES R. ROSE.  
JOHN HARRIS.